

Feb. 5, 1952

H. M. AVERNS ET AL

2,584,779

PRODUCTION OF THREADS OF THERMOPLASTIC CELLULOSE DERIVATIVES

Filed Oct. 15, 1948



Inventors  
Harry Maurice Averns  
Joel Straw

By their attorneys

Hanson and Hanson

## UNITED STATES PATENT OFFICE

2,584,779

## PRODUCTION OF THREADS OF THERMO-PLASTIC CELLULOSE DERIVATIVES

Harry M. Averns, Allesley, Coventry, and Joel Straw, Longford, Coventry, England, assignors to Courtaulds Limited, London, England, a British company

Application October 15, 1948, Serial No. 54,624  
In Great Britain November 12, 1947

3 Claims. (Cl. 18—54)

## 1

This invention relates to the production of threads of thermoplastic cellulose derivatives such as cellulose esters or ethers and in particular cellulose acetate. The term "threads" is used broadly in this specification to include fibres, filaments, threads, yarns, cords and like filamentary materials.

In the production of cellulose acetate and like threads it is well-known to stretch the threads which have been brought to a suitable condition after their formation in order to improve the tenacity. It is also known that the stretching operations generally cause a loss in extensibility, that is the percentage increase in length at the breaking point of the dry thread, so that in general an increase in tenacity is only obtained at the expense of a loss in extensibility. This behaviour is demonstrated by the following figures obtained with one unstretched cellulose acetate thread having a dry tenacity of 1.15 grams per denier and 36 per cent extensibility; on hot stretching this thread 50 per cent the tenacity rose to 2.0 grams per denier and the extensibility fell to 16.0 per cent; on stretching 100 per cent the tenacity was 2.50 grams per denier and the extensibility was 10.0 per cent; on stretching 150 per cent the tenacity was 2.7 grams per denier and the extensibility was 7 per cent; further stretching had little effect on the extensibility which remained fairly constant at 6 to 7 per cent.

It has already been proposed in United States specification No. 1,921,426 to treat artificial silk filaments, the basis of which is cellulose acetate or other cellulose esters or ethers or mixtures thereof, by stretching the dry filaments when they have been brought to the plastic state by heating at a suitable temperature. In the example given in United States specification No. 1,921,426 a thread having an initial dry tenacity of 1.3 grams per denier and an extensibility of 28 per cent is stretched 100 per cent whereupon the tenacity has risen to 2 grams per denier and the extensibility has fallen to 12 per cent.

During normal weaving operations, the threads being woven are generally subjected to varying tension and moreover the tension may at some stages reach a high value. When weaving threads of low extensibility there is consequently a pronounced tendency for the threads to break during the weaving.

The object of the present invention is to produce high tenacity threads of thermoplastic cellulose derivatives which have a sufficient extensibility for normal weaving purposes.

In accordance with the present invention, a

## 2

process for the production of high tenacity threads of thermoplastic cellulose derivatives suitable for weaving comprises the steps of heating preformed threads of the thermoplastic cellulose derivative to a temperature sufficient to render them plastic, stretching the threads at least 50 per cent while they are in the plastic state, and subsequently permitting the threads to shrink at least 8 per cent while they are in a heated plastic state. The stretching and shrinking steps may be carried out while the threads are conveyed through a single heating chamber but are preferably effected in separate heating chambers.

15 In a preferred form of the present invention the stretching of the plastic thread is effected in two stages, the thread being stretched in the first stage at least 40 per cent and in the second stage a lower degree of stretch may be used, for example 30 per cent.

20 The preferred range for the single stretching operation is from 40 to 300 per cent and for the two-stage stretching operation the preferred ranges are from 40 to 150 per cent for the first stage and from 20 to 150 per cent for the second stage. The preferred range for the shrinkage operation is from 10 to 20 per cent shrinkage.

25 The present invention permits the production of threads having a dry tenacity of at least 2 grams per denier and an extensibility of not less than 15 per cent.

30 After the shrinkage of the thread has been effected, it may be advantageous to give the thread an extended passage through the atmosphere before collecting the thread; if desired a current of air at ordinary temperature may also be directed onto the thread. The treatment of the thread with air in this manner allows the thread to become dimensionally stable before it is collected.

35 In carrying out the process according to the invention, the stretching of the plastic thread increases the tenacity and reduces the extensibility and the subsequent shrinking of the thread has little effect on the tenacity but causes an appreciable increase in the extensibility.

40 The process of the invention is preferably conducted continuously with the help of the apparatus diagrammatically illustrated in the accompanying drawing. In this apparatus, three vertical heating tubes 1, 2, 3, preferably electrically heated, are arranged alongside each other and four rotating rollers, 4, 5, 6, 7, for example godets, the diameters and speeds of which are such as to ensure stretching of the thread as it

## 3

passes through each of the first two heating tubes 1 and 2 and shrinkage as it passes through the third heating tube 3. In operation, cellulose acetate thread 8 is drawn from a bobbin 9 and is passed with the aid of fixed guides 10, 11, twice around the first roller 4, then up through the air and with the aid of further guides 12, 13 down through the first heating tube 1 and around the second roller 5 which as shown is on a common driving shaft with, and is of larger diameter than, the first roller 4, then with the aid of guides 14, 15, 16, 17 up through the air and down through the second heating tube 2 and around the third roller 6 which is of smaller diameter than the second roller 5 but is driven at a higher speed of rotation, then once again with the aid of guides 18, 19, 20, 21 up through the air and down through the third heating tube 3 on to the fourth roller 7 which is on a common driving shaft with, but is of smaller diameter than, the third roller 6. The shaft of the first and second rollers 4, 5 as shown is colinear with the shaft of the third and fourth rollers 6, 7. The thread 8 from the fourth roller 7 is given an extended travel through air by means of guides 22, 23, 24, 25, 26 and is then passed to a collecting bobbin 27 of normal construction conveniently with a cap spinning device 28.

The process of the invention is illustrated by the following examples:

## Example 1

The apparatus described above with reference to the drawing was used for stretching dry-spun acetone-free cellulose acetate thread. This thread had a dry tenacity of 1.15 grams per denier and a 36 per cent extensibility. The temperature of the three heating tubes 1, 2 and 3 was approximately 280° centigrade and each tube was 40 inches long. The diameters of the first and second wheels 4 and 5 were designed to give a first-stage stretch of 75 per cent, the diameters and speeds of the second and third wheels 5 and 6 were designed to give a second-stage stretch of 40 per cent, and the diameters of the third and fourth wheels 6 and 7 were designed to give a shrinkage of 12 per cent. The withdrawal speed of the yarn 8 was 75 metres per minute.

After the first stage (75 per cent) stretch the tenacity of the thread was 2.10 grams per denier and the extensibility was 13 per cent. After the second stage stretch the tenacity was 2.40 grams per denier and the extensibility was 10 per cent. After the shrinking step the tenacity was 2.30 grams per denier and the extensibility was 15 per cent.

## Example 2

A single stretching operation was carried out in exactly the same manner as the first stage stretching operation of Example 1, to give a 75 per cent stretch and the shrinking step was designed to give 10 per cent shrinkage.

The stretched yarn, as in Example 1 had a tenacity of 2.10 grams per denier and an extensibility of 13 per cent. After shrinkage the

## 4

tenacity was 2.0 grams per denier and the extensibility was 20 per cent.

In carrying out the above examples, it is not essential to carry out the process continuously. The thread from the second wheel 5 may be collected on a bobbin and subsequently reheated and then stretched and shrunk, or shrunk only, as a separate operation.

The temperature of the stretching tube may be varied, depending on the speed of the stretching, the percentage of stretch and the properties required in the final yarn; for example with cellulose acetate, the temperature may vary from 210° to 360° centigrade according to conditions.

The degree of shrinkage may also be varied if desired to give different extensibilities. Thus in Example 1, using a shrinkage of 15 to 20 per cent, the extensibility may be increased to 17 per cent.

What we claim is:

1. A process for the production of high tenacity threads of cellulose acetate suitable for weaving consisting in heating dry preformed threads of cellulose acetate to a temperature in the range of 210° to 360° centigrade to render them plastic and simultaneously stretching them at least 50 per cent while they are in the dry heated plastic state, whereby the tenacity of the thread is increased to at least two grams per denier and its extensibility correspondingly reduced, and subsequently reheating the dry threads to a temperature within the range of 210° to 360° centigrade to render them plastic and simultaneously permitting the threads to shrink from about 10 per cent to about 20 per cent while they are in the dry heated plastic state, whereby the extensibility of the thread is increased to at least 14 per cent, the plasticity of the thread during both the stretching and the shrinking steps being effected solely by the action of the heat.

2. A process as claimed in claim 1 wherein the stretching is effected in two stages.

3. A process as claimed in claim 2 wherein the thread is stretched from about 40 per cent to about 150 per cent in the first stage and from about 20 per cent to about 150 per cent in the second stage.

H. M. AVERNS.  
J. STRAW.

## REFERENCES CITED

The following references are of record in the file of this patent:

## UNITED STATES PATENTS

| Number    | Name           | Date          |
|-----------|----------------|---------------|
| 1,921,426 | Niogret        | Aug. 8, 1933  |
| 2,142,722 | Dreyfus et al. | Jan. 3, 1939  |
| 2,143,205 | Muller et al.  | Jan. 10, 1939 |
| 2,301,222 | Minich         | Nov. 10, 1942 |
| 2,445,042 | Silverman      | July 13, 1948 |

## FOREIGN PATENTS

| Number  | Country       | Date          |
|---------|---------------|---------------|
| 389,823 | Great Britain | Mar. 20, 1933 |